

# UNITED STATES PATENT OFFICE.

FRANZ HASSSLER, OF HAMBURG, GERMANY, ASSIGNOR TO ADOLF KUTTROFF, OF NEW YORK, N. Y.

## READILY-SOLUBLE TANNING AGENT.

1,390,205.

Specification of Letters Patent. Patented Sept. 6, 1921.

No Drawing.

Application filed July 9, 1920. Serial No. 395,125.

*To all whom it may concern:*

Be it known that I, FRANZ HASSSLER, citizen of the State of Hamburg, residing at Hamburg-Volksdorf, Germany, have invented new and useful Improvements in Readily-Soluble Tanning Agents, for which I have filed applications in Germany, H. 64,719, December 19th, 1913; France, 92,769, July 7th, 1917; Czecho-Slovakia, 18,234, April 1st, 1920; Austria, April 14th, 1920; Sweden, 1,602-20, April 16th, 1920; Hungary, April 17th, 1920; Holland, 14,625, April 23rd, 1920; Norway, 19,995, April 26th, 1920; Denmark, 1,157-20, April 28th, 1920; Belgium, 229,334, May 4th, 1920; Spain, May 20th, 1920, of which the following is a specification.

As is well known, many natural tanning materials are difficultly or incompletely soluble in cold water, thus making the work of the tanner difficult and diminishing the efficiency of the tanning extracts. According to the specification of Letters Patent 1,133,108 such tanning materials can be rendered more soluble by a treatment with soluble phenol condensation products containing at least one salt forming group. In lieu of these condensation products, the specification of Letters Patent 1,216,612 makes, for the same purpose, use of certain aromatic sulfonic acids of an amorphous character, especially of those obtained from naphthalene, formaldehyde and sulfuric acid.

It has now been found that the difficultly soluble parts of tanning materials become readily soluble even in cold water by adding to them sulfonic acids of the higher, at least tricyclic, aromatic hydrocarbons (including

carbazol) such as are found in the less volatile fractions of coal tar. It is only necessary to add the aforesaid materials, or salts thereof, to the tanning extracts or the tanning juices, while hot or cold. The resulting products are readily soluble in water even in a dilute condition. The process is further illustrated by the following example, to which, however, the invention is not confined.

### Example.

100 parts by weight of quebracho extract of about 25° Bé. are mixed with 15 parts by weight of a sodium salt of a sulfonic acid of anthracene, phenanthrene, carbazol, or of mixtures, or of raw products thereof. The mass will quickly get thin and readily soluble in water. The same result as with quebracho extract is produced with other tanning extracts, such as mangrove.

I claim:

1. As a new article of manufacture, readily soluble tanning extracts, comprising a natural tan and a sulfonic acid of an at least tricyclic hydrocarbon.
2. As a new article of manufacture, readily soluble tanning extracts comprising a natural tan, and a salt of a sulfonic acid of an at least tricyclic hydrocarbon.
3. As a new article of manufacture, readily soluble tanning extracts comprising a natural tan, and a sulfonation product of raw carbazol.

In testimony whereof I have hereunto set my hand.

FRANZ HASSSLER.